

## UNITED STATES PATENT OFFICE.

STUART EVAN MACGREGOR, OF WINDSOR, ONTARIO, CANADA.

## ALLOY.

No Drawing.

Application filed December 28, 1921. Serial No. 525,521.

*To all whom it may concern:*

Be it known that I, STUART EVAN MACGREGOR, a subject of the King of England, residing at Windsor, in the county of Essex, 5 Province of Ontario, Canada, have invented certain new and useful Improvements in Alloys, of which the following is a specification.

This invention relates to alloys and it comprises as a new and useful composition of matter, an alloy containing nickel, cobalt, chromium, tungsten and carbon.

The primary use of this alloy is for cutting tools for the machining of cast iron and soft steel at a high rate of speed. It has also been found to be of great value in turning alloy steels containing nickel, molybdenum, and other hardening ingredients. It is especially valuable for use with cast iron 20 and steel articles where the surface is very hard.

The alloy is non-magnetic, non-corrosive and is not readily attacked by any single acid. It will not stain or tarnish under any 25 conditions so far observed. It will take a razor edge and maintain it better than any other similar alloy now known.

The preferred composition of the alloy will consist of nickel about 14 per cent, cobalt about 27 per cent, tungsten about 28 30 per cent, chromium about 31 per cent, and carbon about 1.25 per cent.

An excellent modification of this alloy has the following composition: Nickel about 16 35 per cent, cobalt about 20 per cent, tungsten about 32 per cent, chromium about 32 per cent, and carbon about .98 per cent.

It will be obvious that the percentages of amounts of ingredients set forth in these 40 examples may be varied within reasonable ranges while maintaining the same general characteristics of the alloys obtained in employing such variations as obtained through the use of the percentages presented in these 45 examples.

The function of the nickel appears to be to produce a quality of toughness highly desirable in a cutting tool.

The cobalt has a similar function to that 50 of the nickel in producing the quality of toughness and it also seems to impart the quality of resistance to heat so that the tool will maintain its cutting quality even when at a red heat.

The nickel and cobalt may vary jointly 55 any increase in the amount of cobalt, being accompanied by a corresponding decrease in the amount of nickel. The total percentage of the nickel and cobalt jointly will not vary greatly from 40 per cent of the total amount. 60

The chromium has the function of imparting great hardness to the alloy and it is also an important factor in resistance to corrosion.

The tungsten has the function of increasing 65 the resistance to heat and probably also increasing the hardness of the alloy.

The carbon should not vary greatly from 1 per cent, except for certain special uses referred to later.

It is thought that the nickel, chromium and carbon unite to form a double carbide of nickel and chromium which gives to the alloy its extreme hardness as well as its fine grain and resistance to shock. The alloy 70 is thus probably composed of a solid solution in cobalt and tungsten of a carbide of nickel and chromium.

The alloy is made by melting the ingredients in a crucible in an electric or oil furnace at a temperature of approximately 3600° F. The carbon is included by the addition of boron carbide. The nickel and cobalt are placed in the bottom of the crucible and the chromium placed in a layer over them. The tungsten mixed thoroughly with the requisite amount of boron carbide is then placed upon the chromium and covered with a layer of broken glass.

Upon heating, the glass quickly melts and 80 forms a protecting layer of slag which prevents any loss of carbon and which also protects the hot metal from the oxidizing effect of the air. Any oxides which may be in the mix are removed by the boron. In practice very little, if any, of the boron remains in the finished alloy.

Certain types of arc furnaces may also be used for melting, but those types which are directly to the path must be avoided. This 100 alloy is very sensitive to carbon and therefore anything that tends to make the carbon content hard to control must be avoided.

The alloy should be poured at a heat of about 3600° F. or 200° F. above the melting 105 point. It is very important that the heat of pouring be controlled closely. The alloy should be poured as soon as possible after

melting because upon standing the tungsten tends to separate and to form a semi-fluid mass at the bottom of the crucible.

The alloy should be poured into graphite 5 molds. A small percentage of carbon is taken up by the metal from the graphite so that a casting is obtained with an extremely hard outer or cutting edge and yet with a center sufficiently tough to withstand severe 10 shocks.

For certain purposes, such as valves for acid-proof pumps, where an extremely hard outer edge is not of paramount importance, the melt may be poured into sand molds. In 15 such cases, however, the amount of carbon in the alloy may be increased as much as 75 per cent. With close supervision, an alloy is obtained which is uniform in composition and properties, and which is entirely free 20 from blowholes which in other cutting alloys cause so much trouble.

It will be of course understood that the ingredients as obtained upon the market will contain small percentages of other metals or non-metals, but the addition of these 25 to the alloy in small percentages will not

greatly affect the qualities of the alloy and for certain uses these additional ingredients may even be beneficial.

I claim:—

1. An alloy containing nickel and cobalt, not varying, jointly, widely from 40 per cent of the total, each being present in substantial amount; chromium and tungsten, each not varying widely from 30 per cent of 35 the total; and carbon, in appreciable amount.

2. An alloy containing nickel about 14 per cent, cobalt about 27 per cent, chromium about 31 per cent, tungsten about 28 per 40 cent, and carbon about 1.25 per cent.

3. An alloy in which nickel and cobalt constitute about 40 per cent, chromium and tungsten each about 30 per cent, and carbon about 1 per cent.

In testimony whereof I affix my signature in presence of two witnesses.

STUART EVAN MACGREGOR.

Witnesses:

ARTHUR MINNICK,  
CHARLES W. STAUFFIGER.